

# United States Patent [19]

Gurtler

[11] B 3,925,007

[45] Dec. 9, 1975

[54] **DISPERSE DYE CONCENTRATE WITH SAWDUST**

[75] Inventor: **Peter Gurtler**, 24 Neusatzweg, Therwil, Switzerland

[73] Assignee: **CIBA-GEIGY AG**, Basel, Switzerland

[22] Filed: **Sept. 21, 1972**

[21] Appl. No.: **291,104**

[44] Published under the Trial Voluntary Protest Program on January 28, 1975 as document no. B 291,104.

[30] **Foreign Application Priority Data**

Sept. 30, 1971 Switzerland..... 14209/71

[52] U.S. Cl. .... **8/91; 8/6.5; 8/79**

[51] Int. Cl.<sup>2</sup> .... **D06P 1/46**

[58] **Field of Search** ..... 8/79, 158, 91, 6.5

[56] **References Cited**

## UNITED STATES PATENTS

|         |         |               |        |
|---------|---------|---------------|--------|
| 223,019 | 12/1879 | Vaughan.....  | 8/79 X |
| 253,230 | 2/1882  | Sansone.....  | 8/14 X |
| 253,286 | 2/1882  | Sansone ..... | 8/14   |

|           |         |                 |          |
|-----------|---------|-----------------|----------|
| 1,854,363 | 4/1932  | Aisen .....     | 8/79     |
| 2,000,120 | 5/1935  | Bush .....      | 8/6.5 UX |
| 2,486,562 | 11/1949 | Iamarino.....   | 8/79 X   |
| 3,174,165 | 3/1965  | Dunn et al..... | 8/158    |

## OTHER PUBLICATIONS

Cooley, Practical Science for the Dry Cleaning Industry, 1930, pp. 126-128, 133-138.

*Primary Examiner*—Benjamin R. Padgett

*Assistant Examiner*—B. Hunt

*Attorney, Agent, or Firm*—Joseph G. Kolodny; Edward McC. Roberts; Prabodh I. Almaula

## [57] ABSTRACT

Product for use as a textile processing agent in a textile extraction process comprising from 9 to 75% by weight of the product of a textile processing agent carried on an inert substrate of from 90 to 15% by weight of the product, said substrate being insoluble in the extraction medium having negligible affinity and absorption capacity for said textile processing agent, and from 0 to 10% by weight of the product of an adhesive adapted to assist in bonding the textile processing agent to the substrate and to provide a product substantially free from dust.

**1 Claim, No Drawings**

## DISPERSE DYE CONCENTRATE WITH SAWDUST

The invention relates to new solid preparations containing dyestuff, textile auxiliaries, optical brighteners and/or finishing agents, to a process for their preparation, to their application to the finishing of textile materials by the extraction process, and to the textile material, as an industrial product, treated according to the present invention.

The dyeing of synthetic materials with dispersion dyestuffs is performed usually from a dye liquor containing the dyestuff in very fine dispersion. These processes have the disadvantage that prior to their use the dispersion dyestuffs have to be converted to a form easily dispersible in water according to per se known, but nevertheless intractable and relatively expensive processes utilizing dispersing agents. During the dyeing process, the presence of suitable dispersing agents in the dye liquor is essential for the maintenance of the fine dyestuff dispersion.

The dispersion dyestuffs used for conventional dyeing are offered in a constant tinctorial strength to the consumer. This tinctorial strength is adjusted by the dyestuff manufacturer by incorporation of the appropriate amount of the required dispersing agents and, if necessary, of extenders. All dispersing agents and extenders employed in the production of these dyestuffs preparations must be soluble in the dye liquor.

Synthetic materials can also be dyed by the use of dispersion dyestuffs in the extraction process. With this method of dyeing, the dyestuff does not come into direct contact, as a dispersion in the dye liquor, with the material being dyed, but is deposited in a suitable extraction device and the dye liquor is continuously circulated through it.

By this process, the dyestuff, which is preferably difficultly soluble in the cold state, is dissolved by an extraction process to a degree governed by the solubility of the dyestuff at the temperature of the liquor, and by this process comes into contact with the material to be dyed in dissolved form. Until now this extraction process required suitable preparations which for example also permit the dyeing of commercial quantities in desired shades and are suited for the dyeing of textile materials from aqueous as well as from organic medium.

Accordingly, the technique described above can be used for any type of active substances, such as textile auxiliaries, optical brighteners and finishing agents.

The present invention thus relates to new solid preparations which avoiding the difficulties and disadvantages mentioned are suited for the dyeing, optical brightening and, finishing of textile materials by the extraction process in desired strength. These preparations are characterised in that they contain:

- a. 9 to 75%, preferably 40 to 70%, of at least one active substance,
- b. 90 to 15%, and particularly 80 to 30%, and advantageously 50%, of an inert carrier substance, and,
- c. 0 to 10 percent of an adhesive.

By active agents, above, are meant textile finishing agents such as dyestuffs, textile auxiliaries, optical brighteners and finishing agents.

Preferably dyestuffs, especially dispersion dyestuffs, are used as active substance according to the invention, i.e. those containing no acid, salt-forming, water-solubilising groups. They can belong to the most diverse classes of dyestuffs such as, e.g., the nitro, acri-

done, methine, perinone, naphthoquinoneimine, metal-free, phthalocyanine, heavy-metal-containing phthalocyanine, monoazo, disazo, metal-containing monoazo, metal-containing disazo and anthraquinone dyestuffs; and they can moreover contain a fibre-reactive group. Preferred are monoazo-, disazo-, and anthraquinone dyestuffs. All these dyestuffs are known and can be produced by known methods.

The textile auxiliaries usable according to the invention include softeners; examples of these are:

1. phthalic acid esters such as diethylphthalate, dimethylphthalat, diethylphthalate, dibutylphthalate possibly combined with diethylphthalate, dicyclohexylphthalate, as well as high-molecular phthalic acid esters

15 from decyl and tridecyl alcohol, also mixed phthalic esters such as butyloctyl phthalate, butyldecyl phthalate, butylbenzyl phthalate, diamyl phthalate, diethylhexyl phthalate, dimethyl glycol phthalate and dicapryl phthalate;

20 2. phosphates such as tricresyl phosphate, triphenyl phosphate, triphenyl phosphate combined with tricresyl phosphate and phthalates, diphenylcresyl phosphate, dimphenyl-2-ethylhexyl phosphate, tri-(2-ethylhexyl)-phosphate and tris-(butoxyethyl)-phosphate;

25 3. aliphatic dicarboxylic acid esters, particularly esters of adipic acid and sebacic acid, such as dioctyladipate, didecyladipate, dicapryladipate, dibutylsebacate and butylbenzylsebacate;

30 4. fatty acid esters such as butyl oleate, and butyl stearate;

5. citric acid esters such as acetyltributylcitrate.

All these softeners are known. One of the trademarks under which particularly valuable types are supplied is "Sapamine."

35 A further class of active substances applicable according to the invention is formed by the optical brighteners, especially derivatives of diaminostilbenedisulphonic acid, benzidine, benzimidazole, diimidazole, diphenylimidazolone, phenylbenzothiazole, derivatives of 4-aminonaphthalene-1,8-dicarboxylic acid amide, substituted methylcoumarins, oxazole, oxacyanine-1,3-diphenylpyrazoline derivatives, as well as thiophene derivatives such as 2,5-(benzoxazole-2-yl)-thiophene.

40 Other applicable active substances usable according to the invention are finishing agents such as antistatic agents, dirt repellents and fungicides. In the case of antistatic agents, these are non-ionic, cation-active or anion-active substances. Examples of these are oils, glycols, polyalcohols, polyglycol ethers or quaternary ammonium compounds.

45 Suitable inert carrier substances are inorganic and organic substances which are preferably insoluble in the treatment medium, and which possess a particle size rendering impossible the passage of these substances through the pores of the filter in the extraction process; and which have no or negligible affinity and absorption capacity with respect to the active substance. They are to hold the active agent(s) solely by mechanical means and not change their structure during the treatment process.

50 It is clear that the strength of the active substance can be adjusted to a specific value depending on the percentage thereof present.

55 Examples of suitable inert carriers which may be employed are: diatomaceous earth (kieselguhr in the form of powder), calcium carbonate powder, plastics, sugar, asbestos, silica powder, and wood chips such as, in particular, sawdust, which have a "particle size" of about

3 to 0.6 mm.

Suitable adhesives are nonvolatile solid or fluid products which are not decomposed by the treatment medium but which are preferably soluble therein. They serve to fix the active substance and to prevent any disintegration of the preparation, as well as to ensure the obtainment of the preparation free from dust or containing very little dust.

The following, for example may be used: natural products and synthetic products, e.g., mineral oils, unsatisfiable mineral oils such as "Essotex," oleic acids, amide, carboxymethylcellulose, glycerin, ethylene glycol, and sorbitan fatty acid esters such as sorbitan sesquioleate.

The preparation of the preparations according to the invention follows per se known methods, for example, as follows:

a. the active substance in the formula powder is homogeneously mixed in the dry state with the carrier substance, and, optionally, the obtained mixture moistened in a suitable apparatus, e.g., in a turbulent-chamber coating apparatus, with an adhesive; or

b. the active substance in the form of a powder is mixed dry with the inert carrier substance, and addition is made to this mixture of a solution containing the adhesive either emulsified in water, or dissolved in an organic liquid, e.g., in aliphatic halogenated hydrocarbons such as perchloroethylene, the moist mass subsequently homogeneously mixed and finally dried, or

c. the press cake of the active substance, moistened with water, is homogeneously mixed with a water-soluble or emulsifiable adhesive and the carrier substance; and the obtained mixture subsequently dried.

The same result is obtained when the dry active substance is emulsified with water or mixed with an organic liquid, optionally containing the adhesive in the dissolved state, and the mixture then homogeneously mixed with the carrier substance and dried.

The drying of the preparation is performed in all cases by known methods; e.g., in vacuo at about 50°C, or at elevated temperature around 80°C, e.g. in a heating cupboard or in a roller drier or belt drier.

The preparations have a dust content from zero to a very small amount; they can moreover be produced simply and cheaply, since no special predispersion of the active substance is required.

With the use of granular substances there is obtained a free-flowing preparation of which the dust content ranges from zero to a very small amount. And with the use of pulverulent carrier substances there are obtained lumpy or pulverulent preparations of which the dust content likewise ranges from zero to a very small amount.

The preparations according to the invention are especially suited for the finishing, especially dyeing of textile materials, especially textile materials of synthetic fibers, by the extraction process as described, e.g., in DOS No. 1,938,792.

Suitable synthetic textile materials are, in particular, hydrophobic fibres, such as fibre material made from near high-molecular esters of aromatic polycarboxylic acids, with polyfunctional alcohols such as polyethylene glycol terephthalate fibres, also textured polyester materials, cellulose-di- and -triacetate fibres, and synthetic polyamide fibres, as well as polyacrylonitrile and modified polypropylene. These materials are treated with the said preparations by the extraction process;

e.g., by circulation or an organic liquor such as perchloroethylene, or an aqueous liquor.

Compared with the conventional application processes with dispersion dyestuffs, optical brighteners and finishing agents, the process comprising the use of the preparations according to the invention applying the extraction technique has the following advantages:

no special and expensive fine dispersion of the active substance is necessary; for the production of the preparations, the active substance can be employed in the form of the water-moistened press cake, or as dry powder, and there is no pollution of the effluent since the carrier substance is insoluble in the treatment medium and no dispersing agents are required.

The following examples illustrate the invention, without this being limited by the given examples. The term 'parts' denotes parts by weight, and the temperatures are expressed in degrees Centigrade.

## A. PRODUCTION OF THE PREPARATIONS

### EXAMPLE 1

8 Parts of the dyestuff of the formula



are mixed together with 11 parts of wood sawdust; A solution of 1 part of oleic acid in 14 parts of tetrachloroethylene is then added to the mixture, and the mass homogeneously mixed. A moist loose mass is formed, which is dried in vacuo at 50°. A granular dust-free preparation is obtained containing 40% of dyestuff, 5% of oleic acid and 55% of wood sawdust.

### EXAMPLE 2

If instead of the dyestuff of example 1 or oleic acid equivalent amounts of the dyestuff of the formula



or "Essotex" are used, the procedure being otherwise analogous to that described in Example 1, then a granular, dust-free product is obtained.

### EXAMPLE 3

8 Parts of the dyestuff of the formula



and 11.8 parts of sawdust are mixed together. A solution of 0.2 parts of "Essotex" in 13 parts of tetrachloroethylene is added to the said mixture, and the mass homogeneously mixed. The moist loose mass is dried in vacuo at 50°. A granular product containing negligible dust is obtained.

## EXAMPLE 4

20 Parts of the dyestuff according to Example 3 and 27.5 parts of wood sawdust are mixed together. An emulsion of 30 parts of water and 2.5 parts of "Essotex" is added to the above mixture, and the resulting mass homogeneously mixed. A moist loose mass is obtained, which is dried at 50° in vacuo to obtain a granular, dust-free product.

## EXAMPLE 5

If equivalent amounts of the dyestuff according to Example 2 is employed, with otherwise the same procedure as that in Example 4, then a granular, dust-free product with analogous properties is likewise obtained.

## EXAMPLE 6

4 Parts of the dyestuff according to Example 1 are triturated with a solution of 7 parts of tetrachloroethylene and 0.5 parts of paraffin oil to form a fluid paste. An addition is then made of 5.5 parts of wood sawdust, and the resulting mass homogeneously mixed. A moist loose mass is thus obtained, which is then dried at 50° in vacuo. The resulting product is granular and has a negligible dust content.

## EXAMPLE 7

4 Parts of the dyestuff according to Example 2 are triturated with a solution of 6.5 parts of isopropanol and 0.5 parts of "Essotex" to produce a fluid mixture. An addition is made to this of 5.5 parts of wood sawdust, and the resulting mass further processed as in Example 6. A dyestuff granulate with a low dust content is obtained.

## EXAMPLE 8

4 Parts of the dyestuff according to Example 2 are mixed with an emulsion of 6 parts of water and 1 part of "Essotex." An addition is then made of 5 parts of Kieselguhr powder ("Hyflo"); the whole is homogeneously mixed, and dried at 80° in a thin layer. The resulting product is a soft-granular mass, which can be easily converted into a dust-free powder.

## EXAMPLE 9

2 Parts of the dyestuff according to Example 1 are homogeneously mixed in the dry state with 8 parts of kieselguhr powder ("Hyflo"), without the use of an adhesive. A practically dust-free preparation containing 20% by weight of dyestuff is obtained.

## EXAMPLE 10

A procedure analogous to that described in Example 8 is applied, with the use, however, of the dyestuff according to Example 1, and the addition of equivalent amount of calcium carbonate instead of kieselguhr powder. After drying at 80°, a brittle mass is obtained, which can easily be converted into a dust-free powder.

## EXAMPLE 11

4 Parts of the dyestuff according to Example 1 are mixed together with 5 parts of calcium carbonate powder; a solution of 5 parts of tetrachloroethylene and 1 part of "Essotex" is added, and the whole triturated to form a homogeneous slurry, which is then dried in a thin layer at 50° in vacuo. There is obtained in this manner a soft-granular mass, which can be easily converted into a dust-free powder.

## EXAMPLE 12

If, instead of "Essotex," sorbitan sesquioleate ("Arlacel 83") is used, with otherwise a procedure analogous to that described in Example 11, then here too a soft-granular mass is obtained, which can be readily converted into a dust-free powder.

## EXAMPLE 13

10 4 Parts of the dyestuff according to Example 1 are mixed with 5.5 parts of calcium carbonate powder; a solution of 5.5 parts of tetrachloroethylene and 0.5 parts of oleic acid is then added, and the resulting mass processed as described in Example 11. A soft-granular mass is obtained, which can be easily converted into a dust-free powder.

## EXAMPLE 14

20 7 Parts of the dyestuff according to Example 1 are mixed together with 2 parts of kieselguhr powder ("Hyflo"); a solution of 13 parts of tetrachloroethylene and 1 part of sorbitan sesquioleate ("Arlacel 83") is added, and the whole processed as in Example 11. A soft-granular mass is obtained, which can be easily converted into a dust-free powder.

## EXAMPLE 15

25 4 Parts of the dyestuff according to Example 3 are triturated with 10 parts of a 5% aqueous solution of carboxymethylcellulose. An addition is made to the suspension of 5.5 parts of wood sawdust; the whole is homogeneously mixed, and the somewhat lumpy mass dried at 50° in vacuo. A brittle mass is obtained which crumbles under light pressure to form a dust-free granulate.

## EXAMPLE 16

30 7.4 Parts of the dyestuff of the formula



as a water-moistened press cake having a 54% solid material content, are homogeneously mixed with 1.5 parts 50 of water and 1 part of glycerin. An addition is then made of 5 parts of wood sawdust; the whole is subsequently homogeneously mixed, and dried at 50° in vacuo. A granular, dust-free product is obtained.

## EXAMPLE 17

55 1 Part of 2,5-(benzoxazole-2-yl)-thiophene powder is homogeneously mixed dry with 9 parts of kieselguhr powder ("Hyflo"), without the addition of an adhesive. A practically dust-free preparation containing 10% by 60 weight of optical brightener is obtained.

## EXAMPLE 18

2 Parts of a softener according to the Swiss Pat. No. 320,205 are homogeneously mixed in the dry state with 65 8 parts of kieselguhr powder ("Hyflo"), without the addition of an adhesive. A preparation containing 20% by weight of softener and having a very low dust content is obtained.

**B. APPLICATION OF THE PREPARATIONS IN  
THE EXTRACTION PROCESS**

**EXAMPLE 19**

a. The dyestuff preparation is contained in an extraction holder made from glass fibre; for example a Soxhlet apparatus; the liquor employed is tetrachloroethylene for the dyeing of a knitted fabric made from textured polyester material, Examples 1 to 15, or water for the dyeing of polyamide material with the dyestuff preparation prepared according to Example 16.

A combination dyeing with 0.25% of the dyestuff preparation according to Example 4, 0.55% of the dyestuff preparation according to Example 5, 0.20% of the dyestuff preparation according to Example 6, on a knitted fabric made from texture polyester in tetrachloroethylene, dyed in the "Bowe-solvent-drum-dyeing-machine LFM 12" by the extraction method, produces a dyeing displaying excellent fastness nonstreaky olive to moisture, rubbing, sublimation and light.

b. The preparation according to Example 17 is placed in the glass-fibre holder of a Soxhlet apparatus; polyester Crimplene is then treated for one hour in the extraction process with an aqueous liquor, the liquor containing as carrier 5 ml/l of o-dichlorobenzene, and an emulsifier (ratio of goods to liquor = 1:40). There is obtained on the substrate a very good optical brightening effect.

c. The preparation according to Example 18 is placed into the glass-fibre holder of a Soxhlet apparatus; and polyacrylonitrile fabric (Orlon) treated for one hour, in the extraction process, with a tetrachloroethylene liquor (ratio of goods to liquor = 1:10). There is obtained on the substrate a pronounced softening effect.

15 We claim:

1. A composition for use as a textile dyeing agent in an extraction process consisting essentially of 40 to 70% by weight of a disperse dyestuff carried on 80 to 30% by weight of wood sawdust and 0 to 10% by weight of an adhesive selected from mineral oil, glycerin, sorbitan fatty acid ester or carboxymethylcellulose.

\* \* \* \* \*

25

30

35

40

45

50

55

60

65